

# UNITED STATES PATENT OFFICE.

OSCAR BIRGER CARLSON, OF MÅNSBO, AVESTA, SWEDEN, ASSIGNOR TO AKTIEBOLAGET CARLIT, OF STOCKHOLM, SWEDEN, A CORPORATION OF SWEDEN.

## AMMONIUM-PERCHLORATE EXPLOSIVE.

1,327,985.

Specification of Letters Patent. Patented Jan. 13, 1920.

No Drawing.

Application filed September 25, 1917. Serial No. 193,092.

*To all whom it may concern:*

Be it known that I, OSCAR BIRGER CARLSON, a subject of the King of Sweden, and resident of Månsbo, Avesta, in the Kingdom of Sweden, have invented certain new and useful Improvements in Ammonium-Perchlorate Explosives, of which the following is a specification.

Ammonium perchlorate is as known one of the main constituents of several kinds of modern explosives. Though ammonium perchlorate itself is not explosive, it forms as an oxygen delivering material in connection with combustible additions a powerful explosive.

Such an explosive containing pure ammonium perchlorate is, however, objectionable as it requires, for its explosion a strong impulse from relatively powerful percussion caps or igniters.

At the manufacturing of ammonium perchlorate the impurity of chlorates considered as noxious and originating from the raw materials used at the manufacturing is generally removed. This is effected by separating, for instance by means of centrifugal treatment, the perchlorate from the mother-liquor and the cause of this purification has been, that at using the perchlorate as an explosive it has been supposed that said percentage of chlorate even if it has been very small, should make the perchlorate and thus the explosive unstable and dangerous. By long experiments it has, however, been found that this is not the fact if the percentage of chlorate be only maintained within certain limits.

The present invention refers to an ammonium perchlorate explosive which is made

more sensible to shocks by an addition to 40 the ammonium perchlorate or a percentage left in it, of a certain, small quantity of chlorate for instance potassium, sodium, barium or calcium. The presence of a small quantity of chlorate also increases the velocity of explosion considerably. The quantity of chlorate is proportioned according to the sensibility which is desired to be imparted to the explosive. Said percentage or addition may, however, not be too great, for the reason that if the percentage of moisture in the explosive should increase, a decomposition of ammonium perchlorate and for instance potassium chlorate might take place and ammonium chlorate arise therefrom. The last mentioned material will, however, easily decompose, and is thus dangerous to store or handle. Because of this the chlorate should exist only in small quantities and only amount to between 0.005 and 1% by weight of the quantity of the ammonium perchlorate.

Having now described my invention, what I claim as new and desire to secure by Letters Patent is:

1. Ammonium perchlorate explosive, characterized by the ammonium perchlorate used having a percentage of a chlorate, between 0.005 and 1% by weight.
2. Ammonium perchlorate explosive, characterized thereby that the ammonium perchlorate used has a percentage of chlorate of potassium, between 0.005 and 1% by weight.

In witness whereof I have hereunto signed my name.

OSCAR BIRGER CARLSON.